

## 1

3,078,199

## PROCESS FOR HEAT TREATING TITANIUM-COPPER ALLOY

Charles R. McKinsey, Niagara Falls, N.Y., assignor to  
 Union Carbide Corporation, a corporation of New  
 York  
 No Drawing. Filed Apr. 8, 1959, Ser. No. 804,867  
 1 Claim. (Cl. 148—133)

This invention relates to binary titanium-base alloys and, more particularly to a titanium-copper alloy.

Among the many excellent properties which have interested the metals and chemicals industries in titanium is the high resistance to corrosion possessed by this extremely versatile metal. Titanium is already in competition with nickel-base alloys in corrosion applications, and only production and cost difficulties prevent the full utilization of titanium in many other corrosion fields, such as those dominated by stainless steels. The heretofore imposing challenge of the higher cost of titanium products plus the difficulties involved in casting the extremely reactive molten titanium into suitable shapes have prevented the full exploitation of titanium's valuable property of high resistance to corrosion.

By alloying titanium with other metals the melting point can be reduced and the tendency of the titanium to react with crucibles and molds can also be reduced. For casting operations, it is most desirable to employ a low melting point alloy. In order to significantly reduce the melting point of the reactive metal titanium, however, it is necessary to use relatively large amounts of the alloying additive. The alloying elements which most appreciably depress the melting point of titanium form intermetallic compounds with titanium. It has, therefore, been presumed that embrittlement would result.

It is the primary object of this invention, therefore, to provide a binary titanium-base alloy having a reduced melting point lower than that of the metal titanium, which alloy possesses a useful combination of strength and ductility.

It is another object of this invention to provide a castable binary titanium-base alloy which possesses excellent corrosion resistance.

Other aims and advantages of the invention will be apparent from the following description and appended claim.

In accordance with the present invention, a binary alloy is provided consisting essentially of from about 7 to about 17 percent by weight copper and the balance substantially all titanium.

While in many binary titanium-base alloys the presence of an intermetallic compound may cause embrittlement, the addition of copper in the range specified does not result in a brittle titanium-base alloy, but rather yields a useful material having desirable mechanical and chemical properties.

The alloy produced in accordance with this invention is a hypereutectoid titanium alloy. Despite the presence of a considerable quantity of the intermetallic phase of copper and titanium, the alloy exhibits useful ductility. The alloy is amenable to strengthening and ductility-improving heat treatments that produce a quite stable structure.

The alloy of this invention may be prepared by the same conventional arc-melting techniques which are used for the preparation of other titanium-base alloys. Because of the addition of copper to titanium, the resulting alloy possesses a maximum melting point about 180° C. below that of unalloyed titanium.

In the practice of this invention a binary titanium-

## 2

base alloy was produced from titanium metal having a Brinell hardness number of 72 and containing the following impurities by weight: 0.01 percent carbon, 0.025 percent oxygen, 0.001 percent nitrogen, 0.010 percent hydrogen, and less than 0.005 percent iron. To this titanium base was added copper metal of 99.9 plus percent by weight copper with less than 0.01 percent iron in an amount sufficient to constitute approximately 11 percent by weight of the resulting titanium-copper alloy.

Compacts of this composition, each weighing about 30 grams, were arc-melted by a tungsten electrode in an argon atmosphere, and were finally combined to produce a 120 gram specimen. This was remelted several times to insure complete homogeneity of the alloy ingredients in the cast specimen. The cast specimen was machined for testing and the chips were chemically analyzed. The analysis showed the alloy to be 11.1 percent by weight copper and the balance titanium and incidental impurities.

The machined specimen was then hot rolled to  $\frac{3}{8}$ -inch diameter rod at temperatures within the beta range. The alloy exhibited excellent hot working characteristics in this operation.

Tensile test blanks were prepared for heat treatment by being sealed in heat resistant glass capsules. These

capsules were then evacuated and refilled with argon to a partial pressure of 0.2 atmosphere and then heated in a muffle furnace. The heat-treatment consisted of heating the specimen to 950° C. for 2 hours and water-quenching, followed by heating to 850° C. for 24 hours and

water quenching, followed by heating to 750° C. for 48 hours and water quenching. This heat-treatment consists of heating the alloy at a temperature such that the alloy is within the beta field, followed by cooling below the eutectoid temperature, followed by heating above the eutectoid temperature, cooling below the eutectoid temperature and reheating below the eutectoid temperature.

While this heat-treatment was effective in producing highly stable structures having the excellent properties shown in Table 1, other heat treatments may be used to prevent embrittlement of the alloy and to generally develop the properties of the alloy. A particularly effective heat treatment consists of heating the alloy at a temperature within the beta field, followed by cooling the alloy below the eutectoid temperature, heating the alloy

at a temperature below the eutectoid temperature, and cooling the alloy.

The heat-treated tensile blanks were machined to standard  $\frac{1}{8}$ -inch diameter samples and tested at the usual strain rates for titanium. Stress-strain curves were obtained from which the 0.2 percent offset yield strength and modulus of elasticity were determined. These values are shown below.

TABLE 1

Tensile Test Data

| Yield Strength, 0.2% offset, p.s.i. | Ultimate Strength, p.s.i. | Elongation, Percent in $\frac{1}{2}$ in. | Reduction of area, percent |
|-------------------------------------|---------------------------|------------------------------------------|----------------------------|
| 67,000                              | 93,500                    | 20                                       | 23                         |

The specimens also exhibited a hardness corresponding to a value of 210 in a Vickers hardness test using a 10-kg. load. The modulus of elasticity was  $18.1 \times 10^6$  p.s.i.

Corrosion tests were conducted on samples of the alloy to show its excellent resistance to corrosion and its resulting suitability for use in the chemical industry. These tests were performed on specimens which were heat-treated as described above. The tests were also per-

formed on 316 stainless steel and on a commercial nickel base alloy containing molybdenum and chromium to provide a comparative basis for the tests. In these tests, the alloy samples were weighed, immersed in boiling 30 percent ferric chloride for from 48 to 60 hours, removed, washed and weighed again to determine the amount of corrosion. Similar alloy samples were tested in the same manner in 30 percent nitric acid maintained at a temperature of 190° C. The corrosion rates were calculated for all the samples and are reported as mils penetration per year in Table 2.

TABLE 2  
Comparative Corrosion Resistance

| Sample                                           | Corrosion Rate, Mil penetration per year |                                  |
|--------------------------------------------------|------------------------------------------|----------------------------------|
|                                                  | in 30% HNO <sub>3</sub> at 190° C.       | in boiling 30% FeCl <sub>3</sub> |
| 11.1% Copper-Titanium Alloy                      | 129                                      | 2.26                             |
| 316 Stainless Steel                              | 1,690                                    | Dissolves                        |
| A commercial Ni-Base alloy containing Mo and Cr. | Dissolves                                | Do.                              |

It is apparent from the above results that the corrosion resistance of this alloy is far superior to such common corrosion resistant alloys as 316 stainless steel and a commercial nickel-base alloy containing molybdenum and chromium.

In summary, an alloy can be prepared in accordance with the disclosure herein which will exhibit a yield strength in excess of 60,000 pounds per square inch; an

ultimate strength in excess of 85,000 pounds per square inch, an elongation of about 20 percent, and a corrosion rate in 30 percent nitric acid at 190° C. of less than 200 mils penetration per year.

5 The description of the invention above has been in terms of its specific embodiments. Modifications and equivalents will be apparent to those skilled in the art and this disclosure is intended to be illustrative of, but not necessarily to constitute a limitation upon, the scope 10 of the invention.

What is claimed is:

A process for producing a titanium-base alloy characterized by useful ductility comprising preparing an alloy consisting essentially of about 11 percent by weight 15 copper and the balance titanium and incidental impurities, heating the alloy at a temperature of about 950° C. for about 2 hours, quenching the alloy in water, thereupon reheating the alloy at a temperature of about 850° C. for about 24 hours, quenching the alloy in water, and 20 reheating the alloy at a temperature of about 750° C. for about 48 hours and quenching the alloy in water.

References Cited in the file of this patent

McQuillan: Institute of Metals, vol. 79 (1951), page

25 73.

Harrington: AIME Transactions, vol. 124 (1937), page 172.

Hansen: Constitution of Binary Diagrams, 2nd edition, published by McGraw-Hill Book Co.

30 Holden et al.: "Journal of Metals," vol. 7, pages 117-125, January 1955 (pages 117, 119 and 123 are relied on).